

## UNITED STATES PATENT OFFICE

JAMES BADDILEY, OF BLACKLEY, MANCHESTER, ENGLAND, ASSIGNOR TO BRITISH DYESTUFFS CORPORATION, LIMITED, OF BLACKLEY, MANCHESTER, ENGLAND

## APPLICATION OF AZO DYES

No Drawing. Application filed December 3, 1927, Serial No. 237,592, and in Great Britain December 10, 1926.

This invention relates to certain improvements which I have discovered in connection with the application of the azo dyes which can be made by combining the diazo compound of para-nitroaniline ortho-sulphonic acid, with any middle component, re-diazotizing and combining, either in alkaline or acid solution, with 2-amino-5-naphthol-7-sulphonic acid or its N-alkyl, aryl or acyl derivatives. These dyestuffs have been known for a considerable time and have been described as dyestuffs for dyeing cotton, but they have never come into use in the dyeing industries. I have now discovered that these dyestuffs possess a good affinity for artificial silk fibres composed of regenerated cellulose, and in particular that they have the valuable property of giving even dyeings on fabrics made from these regenerated cellulose silks. Various shades of blue can be obtained. These dyestuffs may be represented by the following formula:



wherein R<sub>1</sub> represents a divalent naphthalene or benzene residue and R represents hydrogen, alkyl, aryl or acyl group.

The application of these dyestuffs for dyeing regenerated cellulose silks has not hitherto been known, and the process according to my invention, whereby level blue shades on these fibres by the use of hitherto useless dyes can be obtained, is therefore of considerable technical value. Those who are concerned with the dyeing of goods made from regenerated cellulose silks, for example from viscose silk, are well aware that these fibres present special problems in dyeing because the avidity of the silk for dyestuffs is frequently

irregular. As a result of this irregular avidity of the silk, the dyeings obtained frequently come out very uneven in depth of shade. This is particularly the case when the dyeing is carried out with the usual substantive blue dyestuffs, for example with the bright blue dye obtained by coupling dianisidine with two molecules of 1:8-aminonaphthol-2:4-disulphonic acid. The dyeings which are obtained according to my invention are notably level in depth of shade, and I have therefore by my invention introduced a valuable technical application for dyestuffs which have hitherto not been of service in the dyeing industries. The dyeing process is illustrated by the following example, but it must be understood that I do not limit myself to the conditions named therein:

The dyebath is made up from 3000 parts of water, a little soap and about 20 parts of Glauber's salt and one part of the secondary disazo dye obtained in the known manner by combining diazotized para-nitro aniline-ortho-sulphonic acid with alpha-naphthylamine, re-diazotizing and combining with 2-amino-5-naphthol-7-sulphonic acid in alkaline solution. One hundred parts of the silk material to be dyed is entered into the bath, after which the bath is heated up nearly to the boil and the dyeing carried out nearly at the boil for about one hour. The goods are then removed, rinsed off and dried, the resulting dyeings being a level blue shade. If in the above example, a dye prepared by substituting a sulphonated alpha-naphthylamine in place of alpha-naphthylamine is used (the dye in this case having as free acid the probable formula



wherein hydrogen, alkyl, aryl and acyl groups are all represented by R) an equally advantageous dyed product is obtained.

Further examples illustrative of my invention are quoted in the following table:

| Secondary disazo colour from diazotized para-nitroaniline-ortho-sulphonic acid combined with— |                                                               | Shade on viscose silk |
|-----------------------------------------------------------------------------------------------|---------------------------------------------------------------|-----------------------|
| Middle component                                                                              | End component                                                 |                       |
| 10                                                                                            | Alpha-naphthylamine                                           | Blue                  |
| 15                                                                                            | Alpha-naphthylamine                                           | Blue                  |
| 20                                                                                            | m-amino-p-cresol-methyl ether                                 | Reddish blue          |
| 25                                                                                            | Do.                                                           | Bright blue           |
|                                                                                               | 2-phenylamino-5-naphthol-7-sulphonic acid (coupled alkaline)  | Blue-violet           |
|                                                                                               | 2-acetylaminio-5-naphthol-7-sulphonic acid (coupled alkaline) | Blue                  |

What I claim and desire to secure by Letters Patent is:—

1. The process of dyeing regenerated cellulose silks in level blue shades, which comprises dyeing such a silk with secondary disazo dyes obtained by coupling diazotized para-nitroaniline-ortho-sulphonic acid with an amine having the following formula  $H_2N-R_1$  where  $R_1$  represents a naphthyl or phenyl residue, the said amine being capable of coupling with diazo compounds to form a diazotizable amino azo compound, rediazotizing and coupling with a compound of the type



45 in which hydrogen, alkyl, aryl and acyl groups are all represented by R.

2. The process of dyeing regenerated cellulose silks in level blue shades which comprises dyeing such a silk with a secondary disazo dye obtained by coupling diazotized para-nitroaniline-ortho-sulphonic acid with alpha-naphthylamine, rediazotizing the product and coupling with a compound of the type



60 in which hydrogen, alkyl, aryl and acyl groups are all represented by R.

3. The process of dyeing regenerated cellulose silks in level blue shades which comprises dyeing such a silk with the secondary disazo dyestuff obtained by coupling diazotized p-

nitroaniline-o-sulphonic acid with alpha-naphthylamine, rediazotizing the product and coupling with 2-amino-5-naphthol-7-sulphonic acid.

4. The process of dyeing regenerated cellulose silks in level blue shades which comprises dyeing such a silk with the secondary disazo dyestuff obtained by coupling diazotized p-nitroaniline-o-sulphonic acid with alpha-naphthylamine, rediazotizing the product and coupling with 2-amino-5-naphthol-7-sulphonic acid in alkaline media.

5. Regenerated cellulose silks dyed in level blue shades with a dye having the formula in the free acid form of



where hydrogen and a sulphonic group are represented by X, and in which hydrogen, alkyl, aryl and acyl groups are all represented by R.

6. Regenerated cellulose silks dyed in level blue shades with a secondary disazo dye obtained by coupling a diazotized para-nitroaniline-ortho-sulphonic acid with an amine having the probable formula



wherein  $R_1$  represents a phenyl or naphthyl residue, said amine being capable of coupling with diazo compounds to form a diazotizable amino azo compound, rediazotizing and coupling with a compound of the type



105 in which hydrogen, alkyl, aryl and acyl groups are all represented by R.

7. Regenerated cellulose silks dyed in level blue shades with a disazo dye obtained by diazotizing para-nitroaniline-ortho-sulphonic acid with an amine of the class consisting of alpha-naphthylamine and meta-amino para-cresol-methyl ether, rediazotizing and coupling with a compound of the type



115 wherein  $R_2$  represents hydrogen, ethyl, phenyl or acetyl groups.

In testimony whereof I affix my signature.  
JAMES BADDILEY.